

March 5, 1935.

G. S. ROWELL

1,992,965

METHOD OF PRESERVING COLLOID FILMS

Filed Sept. 19, 1932



*Inventor,  
George S. Rowell,  
by Paluto, Lehman & Woodberry.  
All rights reserved.*

## UNITED STATES PATENT OFFICE

1,992,965

## METHOD OF PRESERVING COLLOID FILMS

George S. Rowell, Cleveland, Ohio, assignor to  
Multigraph Company, Wilmington, Del., a cor-  
poration of Delaware

Application September 19, 1932, Serial No. 633,823

8 Claims. (Cl. 95—8)

This invention relates to the preparation and preservation of the actinic sensitiveness of chromated colloid films, and it comprises coating a freshly dried film of chromated colloid on a suitable support in a non-actinic light with a transparent film of water-insoluble, but preferably water-permeable, waxy material, whereby the actinic sensitiveness and the surface continuity of the chromated colloid film is maintainable.

- 10 Light-sensitive chromated colloid films have been extensively used in the graphic arts; and, whether the colloid, sensitized by bichromates or chromates, was glue, gelatin, albumin or other colloid, it was invariably the custom to use the prepared material within a few hours after it was dried. Not only would the actinic sensitiveness diminish with time, but the resistance to swelling of the light-hardened protein progressively diminished with the time elapsing between 15 drying the sensitive layer and the development thereof. Furthermore, if a film of the chromated colloid were dried to a moisture content much below that at which it first became palpably dry, it exhibited a tendency to shrink and 20 crack. This tendency to form minute surface cracks upon excessive drying is accentuated in films of uneven thickness, such as inevitably result from flooding a grained lithographic plate with a thin film of chromated colloid.
- 25 As is well recognized in the art, a chromated colloid film must be relatively thin in order that it may be hardened through to the base support by the action of light. The depressions of the grained surface of a lithographic plate therefore produce appreciable variations in the thickness of a film on such surfaces, and in consequence when such a film shrinks and cracks, the cracks are determined by and correspond to the variations in thickness produced by the grain de- 30 pressions, and hence are distributed over the entire plate surface. Even if the actinic sensitiveness of a dry chromated colloid film were maintained, these minute cracks would render the film unfit for lithographic reproduction.

- 35 40 45 50 55 Lithography depends upon the immiscibility of water and oil and the chromated colloid light-hardened image surfaces serve as a base for the ink which is to be transferred to paper. The non-printing areas of the plate must be maintained free of greasy ink and readily wettable by water and therefore must be entirely freed of the chromated colloid not an essential part of the image. In order to facilitate development of a light-hardened colloid image, it is essential that the operator should be able to visually de-

termine when all the non-hardened colloid has been washed off the non-image areas of the plate. It is also desirable to condition the light-hardened or retained colloid constituting the image for grease receptivity by contact of the same with a so-called developing ink before developing the image with water. If, however, the chromated colloid film has been subjected to conditions conducive to excessive loss of moisture, shrinkage and consequent cracking occurs, as stated, and upon treating the exposed surface with developing ink, this ink passes through these cracks and reaches the surface of the underlying plate. Where these cracks underlie non-printing areas the effect of such contact of the plate by the developing ink is disastrous as each inky delineation of a crack on the plate will ultimately pick up enough printing ink to record itself in the highlights of the printed image.

It is an object of my invention to so prepare and protect a dried chromated colloid film on a planographic printing plate as to permit of the storage of such plate for an indefinite period without appreciable loss of actinic sensitivity and without detrimental surface cracking. Other objects and advantages will become apparent from its more detailed description, and from an examination of the accompanying drawing which shows in exaggerated cross section a plate bearing an actinically sensitive film protected in accordance with my invention.

It is well known in the art that the effect of the exposure of a chromated colloid film to light depends not only upon the intensity of the light and the duration of the exposure but upon the elapsed time between exposure and development. The effect of a given exposure increases with such elapsed time. It is also well known that a chromated colloid film becomes light-sensitive only when dry.

I have discovered that if I dry a film of chromated colloid supported on the surface of a planographic printing plate in non-actinic light, that is, a light which produces no measurable hardening effect on the film regardless of the time which may elapse between drying and developing, and after drying until the last visible traces of moisture have disappeared and the film is palpably dry, I coat the film with a thin layer of a water-insoluble transparent waxy material and then seal the so dried and protected film in a light-tight envelope; the actinic sensitiveness of the film will persist substantially undiminished, if not indefinitely, at least for a year or more, and that upon removal of the waxy film

by means of a suitable solvent it will be found that the integrity of the surface continuity has also persisted, i. e., the surface will be found to be free from detrimental cracks.

5 A suitable water-insoluble waxy film may be obtained from a solvent solution of wax, paraffin, or the like, but obviously such a film must be removed by the use of a suitable non-aqueous solvent before the underlying colloid may be developed with water.

10 I have further discovered as part of this invention, however, that all the advantages of the waxy film above described, but without the disadvantages attendant upon the necessity for the 15 removal of this waxy coating by a non-aqueous solvent, may be obtained by the use of a film which, though water-insoluble, is water-permeable. Any such water-insoluble film, which is however sufficiently water-permeable to permit 20 water to get at and dissolve the underlying unhardened chromated colloid and which is readily carried away with and by the dissolving colloid, i. e., which is not inherently tough, is suitable 25 for my purpose. Preferably I use materials which tend to remain firmly adherent to the light-hardened image area. The following formula is illustrative of compositions suitable for my purpose:

|            | Ounces |
|------------|--------|
| 30 Beeswax | 1 1/2  |
| Tallow     | 3      |
| Turpentine | 20     |

35 I have also discovered that I may avoid the use of organic solvents by emulsifying wax alone or preferably wax and tallow in water, coating the dried colloid film with such emulsion and by subsequently removing the aqueous phase by desiccation.

40 Not only should the drying of the chromated colloid film be carried out in the dark, or at least in a non-actinic light, but the subsequent coating operation should also be so carried out as at all times to avoid subjecting the film to any light capable of exerting a hardening action 45 on the colloid. I find that the usual whirling apparatus is a satisfactory means of obtaining both the primary light-sensitive coating and the superimposed protective waxy coating. In general I find it desirable to apply as 50 thin a film as will yield an unbroken continuous surface, except in the case of the emulsion where a film of the order of two or three ten-thousandths of an inch is desirable. The protected light-sensitive film of this invention may, 55 after protracted storage, be exposed and de-

veloped in the usual way except when the protective coating is water impermeable, in which case it must be removed by a suitable solvent before development of the colloid film with water. And due to the fact that cracking of the film has been prevented, the non-printing areas will be free from the objectionable inky delineations thereof.

5 By the expression "waxy", as used herein is comprehended all those materials, including 10 strictly chemical waxes, which have in common the physical characteristic of unctuousness.

I claim:

1. A method of preserving actinically sensitive chromated colloid films, comprising as steps 15 treating the freshly dried film with a coating of water insoluble but water permeable waxy material and drying the same.

2. A method of preserving actinically sensitive chromated colloid films, comprising as steps 20 treating the freshly dried film with an emulsion coating of water insoluble but water-permeable waxy material and drying the same.

3. A method of preparing freshly dried light sensitive chromated colloid films, on planographic printing surfaces, comprising as a step 25 preserving the surface with a chromated colloid, drying, coating with a water insoluble waxy material, and, when ready for use, exposing the film through said coating and developing the 30 required image in said film, the coating remaining adherent to the light-hardened image area.

4. A method of preparing freshly dried light sensitive chromated colloid films, on planographic printing surfaces, comprising as a step preserving 35 the surface with a chromated colloid, drying, coating with a water insoluble but water permeable waxy material, and, when ready for use, exposing the film through the coating and developing the required image in said film.

5. Actinically sensitive chromated colloid films, characterized by being palpably dry and by having a coating of water insoluble waxy material.

6. Actinically sensitive chromated colloid films, characterized by being palpably dry and by having a coating of water insoluble but water permeable waxy material.

7. A planographic printing surface having a light sensitive film of chromated colloid and a 50 coating of water insoluble waxy material.

8. A planographic printing surface having a light sensitive film of chromated colloid and a coating of water insoluble but water permeable waxy material.

GEORGE S. ROWELL.

55